

Dec. 20, 1960

V. TULAGIN ET AL

2,965,484

MIXED PACKET PHOTOGRAPHIC EMULSIONS

Filed March 26, 1956



Fig. I



Fig. II

VSEVOLOD TULAGIN  
ROBERT D. JACKSON  
INVENTORS

Henry W. Confer  
Edward P. Gibbons  
ATTORNEYS

# United States Patent Office

2,965,484

Patented Dec. 20, 1960

1

2,965,484

## MIXED PACKET PHOTOGRAPHIC EMULSIONS

Vsevolod Tulagin and Robert D. Jackson, Binghamton, N.Y., assignors to General Aniline & Film Corporation, New York, N.Y., a corporation of Delaware

Filed Mar. 26, 1956, Ser. No. 573,799

7 Claims. (Cl. 96—55)

The present invention pertains to hydrophobic silver halide grains, said grains dispersed in a highly non-water miscible liquid, water-sensitive or hydrophilic colloidal carriers containing such dispersions, and light sensitive emulsions containing a matrix of a water-sensitive or hydrophilic colloidal medium having dispersed therethrough immobile packets of a highly non-water miscible solvent surrounding hydrophobic silver halide grains with associated sensitizers and, if desired, color formers capable of yielding a dye image complementary in color to the light rays for which such hydrophobic silver halide grains are respectively sensitized, and methods for producing said grains and compositions.

Many years of effort have gone into the immobilization of sensitizers, color formers and silver halide grains in photographic carriers, such as gelatin, polyvinyl alcohol and the like. The purposes behind the immobilization or non-migration of color formers and/or sensitizers, per se, are rather obvious at this stage of the photographic art and need be touched upon but lightly.

It is usual in the manufacture of light sensitive color materials to employ in the photographic emulsions thereof color formers reactive with another agent, such as an oxidized primary aromatic amino developer, to form dye images. It is equally the practice to locate the color formers leading to the colored images in different layers of the color material. Were such coupler to wander from layer to layer, color degradation and distortion would inevitably ensue. This problem has been solved by making the color formers "substantive" to the colloidal carrier, by including in the color former a long aliphatic chain, or by associating the color former with a non-migratory high molecular weight relatively high boiling oil, such as tricresyl phosphate or the like.

The migration of sensitizer from layer to layer of color film has not been a particular problem. However, a real problem arises if this phenomenon is permitted to ensue in so-called "variable contrast" paper. In such materials, two photographic emulsions of quite different contrast, each sensitized to different regions of the spectrum, are intermixed. The contrast of the image of such papers is controlled by the color of the exposing light. It is imperative in such materials to avoid migration of the sensitizers from grain to grain and also so-called "contagious development" wherein one exposed grain will cause several unexposed grains to become developable. In other words, it is essential that each emulsion function completely independently of the others present.

A number of suggestions leading to the solution of this problem have been made. These involve the employment of a specific sensitizer structure, the addition of the silver halide to dye sensitized emulsions followed by mixing the so-prepared emulsion with the other (U.S.P. 2,411,096) and the use of perhalogenated salts, such as sodium perchlorate (U.S.P. 2,239,699).

For numerous years, color film has been prepared and vended in the form of integral monopacks. The manufacture of such products is intricate and time consuming

2

involving, as it does, the laying down of a number of light sensitive balanced coatings, one upon the other. Furthermore, sensitivity or speed is a factor to be struggled with, due to the distance apart of the various sensitized layers. As a result, the art has been continuously "shooting" for the optimum, to wit, a color film with only one sensitized layer containing the sensitized grains needed for the three primary colors. This material, to which considerable research and development have been devoted but which, nevertheless, is still in the dream stage, is known in photographic parlance as "mixed grain" film.

Were a product of this type to be commercially realized it would have the following manifest and very important advantages over present day monopacks:

- (1) Ease of preparation, i.e., decrease in the number of coating steps;
- (2) Greater control in the manufacturing process;
- (3) Superior quality in light sensitivity and resolution due to the close proximity of the sensitized grains; and
- (4) Simplification in processing.

It is no wonder, therefore, that time and money have been poured into the creation or realization of a product permitting the attainment of these desiderata.

A full gamut of photographic procedures has been run in efforts to devise a commercial "mixed grain" film. These have ranged from the use of hardened, differently sensitized emulsion granules, first suggested by Wendt in 1937 (U.S.P. 2,168,182) and later in U.S.P. 2,618,553 to the formation of "individual packets" of silver halide grains, sensitizer and, if desired, color former. Most of the work has been in the latter category, all of which has been bottomed on endeavors to immobilize the silver halide grains in the emulsion so that they are alienated from their associates and, hence, capable of functioning as individualists rather than as part of the herd.

One of the early moves in this direction was keyed to the addition of modifiers of high molecular weight having the ability to dissolve the color former imbibed to the silver halide grain, whereby color former association with the modifier would prevent its diffusion from the colloidal carrier. To this end, it was proposed to employ such high molecular weight compounds as polyvinyl alcohol, polyvinyl phthalate, gum arabic and the like (U.S.P. 2,289,803).

Subsequently, it was decided to produce hydrophobic emulsions (water repellent) and, in U.S.P. 2,304,939, it was suggested that the colloidal carrier for the light sensitive salts be collodion rather than gelatin. This theory was elaborated on in U.S.P. 2,284,877 which suggested that the silver halide be precipitated with color former and/or sensitizer in the presence of a water insoluble resin, such as amber, shellac, and the like, and a solvent therefor. The mixture thus obtained would then be dispersed in a water permeable colloid, such as gelatin. It was recognized, however, that the speed of this material would be quite low and the further suggestion was made that gelatin should be present at the time of precipitation or formation of the silver halides.

It was later proposed to use zein as the peptizing agent (colloid) in the formation of "mixed grain" packets. In this procedure, the silver halide is formed in zein to produce oil soluble packets which are then dissolved in benzyl alcohol. The resulting solution, to which sensitizers and/or color formers may be added, is then dispersed in a water receptive carrier, such as gelatin (U.S.P. 2,563,791). This procedure was claimed to be improved upon by the use of  $\gamma$ -phenyl propyl alcohol in lieu of benzyl alcohol as the solvent (U.S.P. 2,490,749).

The next phase witnessed the formation of packets by use of a water soluble colloid, capable of being rendered

water insoluble, and the dispersion of the resulting packets in a water permeable colloid, such as gelatin or polyvinyl alcohol. In this method, the silver halide grains are dispersed in a colloid, such as alginic acid, oxidized cellulose or the like, sensitizers and color formers added and the whole made water insoluble by treatment with an alkaline earth metal salt, such as calcium chloride, calcium acetate and similar compounds. The insolubilized product is then dispersed in a water permeable colloid to form individual sensitive grains immobilized in the aqueous phase (U.S.P. 2,548,526).

A further advance in the "packet" concept was claimed in British Patent 711,488 and U.S.P. 2,698,795 and U.S.P. 2,698,796, which turned upon the use, for enveloping the silver halide grains with associated sensitizers and color formers, if desired, of a copolymer of styrene and maleic anhydride, on the one hand, and a water soluble polymer containing salt forming acid groups, on the other hand, such as a copolymer of methacrylic acid and methyl- $\alpha$ -methacrylate. The colloidal carrier in this system is gelatin in which the silver halide is precipitated.

Another modification of the "packet" system appears in British Patent 718,404, in which separate silver halide emulsions are formed, hardened and then dispersed in a water insoluble cellulose ether and a partially water miscible solvent, such as acetone or the like.

Attempts have also been made to remove the gelatin from normal photographic gelatin emulsions and to disperse the isolated silver halide in colloidal carriers, such as polyvinyl alcohol or carboxymethyl cellulose. However, it has not been possible to isolate the silver halide grains from a gelatin emulsion and to disperse them in an oily or a water insoluble medium, for the reason that the silver halides of normal photographic emulsions are hydrophilic. By "hydrophilic" is meant that the silver halides are preferentially wetted by water and even though obtained in a dry state, if dispersed in a water insoluble medium, would leave such medium and go into water or an aqueous solution if shaken therewith.

Despite the great volume of work devoted to the packet system for mixed grain emulsions, the fact remains that, as yet, there is no known commercially available light sensitive material which invokes these principles. Thus, in British Patent 711,488 it is stated:

"Prior processes employing mixed packet emulsions have not been successful either because it was impossible to secure colour separation with them, that is, effectively to prevent colour formation around unexposed silver halide grains, or because the coloured particles formed in the process were too grainy."

The pattern followed by prior operators to effect and maintain the isolation of silver halide grains in packets is self-evident from the above résumé. As previously noted, the silver halide in normal photographic emulsions has an inherent propensity to segregate in the emulsion. In the packet system generally followed, the idea has been, not to divest the silver halide grains of this natural propensity, but rather to imprison or entrap the grains through a hit or miss manner in a cell or envelope of a body foreign to the carrier matrix, such as a water insoluble or water soluble natural or synthetic resin.

We have now discovered that we can isolate silver halide grains in a water permeable matrix by rendering such grains hydrophobic so that their tendency to segregate or coalesce is eliminated. Once the grains have been made hydrophobic, they are amenable to dispersion in an oily non-water miscible liquid and, if desired, with sensitizers, color formers and other photographic emulsion adjuncts to form a packet readily dispersible in a water permeable colloid. Surprisingly, each packet remains fixed or isolated in its assigned sphere in the

matrix and is capable of functioning as an individual entity.

5 The isolation of silver halide grains by rendering the grains hydrophobic, dispersions of such grains in a highly, non-water miscible solvent, water-sensitive or hydrophilic colloidal carriers containing such dispersions, and light sensitive emulsions containing said dispersions along with associated sensitizers and, if desired, color formers, constitute the purposes and objects of our invention.

10 Our invention is predicated upon the realization that silver halide grains in normal photographic emulsions are surrounded by an envelope of adsorbed gelatin which cannot be removed without disrupting the crystal and destroying the photographic properties thereof. We have ascertained, and these constitute the critical factors of our procedure, that such gelatin envelope is amenable to chemical treatment with a compound containing a hydrophobic radical and a group reactive with amino compounds to produce hydrophobic silver halide grains dispersible in an oily, non-water miscible liquid. Dispersions of such hydrophobic grains when emulsified in gelatin solutions or the like are completely immobile therein, a fact readily demonstrated by microscopic examination. 15 For example, if silver halide grains surrounded by a gelatin hull are dispersed in phenyl ethyl alcohol and the resulting dispersion is then emulsified in gelatin, the microscope reveals that the silver halide grains leave the solvent and wander into the gelatin matrix. A similar 20 examination of a dispersion produced as above, with our hydrophobic system, establishes that the grains refuse to leave the solvent for the gelatin.

25 The preparation of highly sensitive emulsions containing the hydrophobic silver halide grains begins with a normal silver halide gelatin emulsion. Such emulsion is subjected to enzymatic hydrolysis to destroy the excess gelatin and, to this end, there may be employed any number of enzymes, such as pectinase, trypsin and the like. The enzymatic action is permitted to continue until 30 the silver halide can be readily decanted. It has been shown by Dr. Frank Hamm, J. Applied Phys. 24, 1495-1513 (December 1953), that such enzymatic digestion does not disrupt the gelatin envelope which surrounds each silver halide grain. It has been established by us 35 that such enzymatic digestion does not alter the photographic properties of such grain.

40 After the excess gelatin has been destroyed, the silver halide grains are separated from the aqueous medium by decantation, filtration or centrifugation. The isolated solid is re-suspended in a normally liquid (i.e., liquid at room temperature) inert non-aqueous organic solvent, such as acetone, methylethyl ketone, benzene, ethyl acetate or the like, and thoroughly washed to remove 45 any residual free water. The solid in such solvent is then subjected to the action of a chemical reagent capable of rendering the surface of the gelatin envelope hydrophobic.

50 In its broadest sense the latter treatment consists in closely associating the gelatin envelope of each silver halide grain with a hydrophobic moiety (see Schwartz-Ferry, Surface Active Agents, Interscience Publishers, Inc., New York, 1949, pages 17-20), preferably, a long aliphatic chain, i.e., containing ten or more carbon atoms. To this end, there may be employed compounds 55 containing a hydrophobic radical, on the one hand, and a group readily reactive with amines, on the other hand, such as long chain acid anhydrides, acid chlorides, sulfonyl chlorides, isocyanates or chlorocarbonates. Such long chain aliphatic compounds are those normally employed in modifying surface properties. Examples of such compounds are tetradecyl isocyanate, hexadecyl isocyanate, myristyl isocyanate, myristic anhydride, palmityl anhydride, myristoyl chloride, palmitoyl chloride, stearoyl chloride, myristylsulfonyl chloride, palmitylsulfonyl chloride, stearylsulfonyl chloride, decylchloro-

carbonate, hexadecylchlorocarbonate, tetradecylchlorocarbonate, and the like.

The treatment with these reagents is effected in normally liquid, inert organic solvents, such as, acetone, benzene, ethyl acetate, butyl acetate, methylethyl ketone and the like.

It is our theory that the reagents in question react with the gelatin hull to form either a covalent or coordinate bondage therewith. This theory is predicated on a number of factors, to wit:

(1) The activity of the anhydride, acid chloride, sulfonyl chloride, isocyanate or chlorocarbonate groups insofar as amino groups are concerned and their ability to react therewith to form amides;

(2) The proposal in U.S.P. 2,179,244 to react gelatin with, inter alia, long chain acid chlorides;

(3) The fact indicated above that the silver halide, after treatment, is hydrophobic in the true sense of that term; and

(4) The silver halide grains are not rendered hydrophobic in the event that the reagent employed is relatively inert to amines, i.e., a carboxylic acid, per se, such as myristic acid.

In any case, if our theory of chemical conversion be incorrect, we are certain that a close physical or chemical association takes place between the involved reactants and the gelatin hull, which association leads to the formation of the hydrophobic silver halide grains. Typically, we have treated silver halide grains subjected to enzymatic digestion with myristic acid under the same conditions as such grains were treated with myristic anhydride. The grains so treated, when dispersed in phenyl ethyl alcohol and emulsified in gelatin, refused to remain in the solvent and migrated to the gelatin. It is thus evident that the association necessary to effect the desired hydrophobic condition cannot be obtained without using a compound having a grouping with a very marked tendency to react with amino groups to form amides.

After the treatment to impart hydrophobic character to the silver halide grains, the excess of the hydrophobating reagent is removed by washing with an organic solvent, such as acetone, and gradually replaced with another organic solvent which is to be the final carrier for the transformed silver halide and which is an oily, non-water miscible liquid, such as benzyl alcohol, phenyl ethyl alcohol,  $\gamma$ -phenylpropyl alcohol or the like, phthalic acid esters, i.e., dibutyl phthalate, di- $\beta$ -ethoxyethyl phthalate, tricresyl phosphate, triphenyl phosphate, or a combination of such solvents.

The silver halide grain in such solvent is now added to non-aqueous solutions of color formers, sensitizing dyes, stabilizers and other adjuncts usual in the manufacture of photographic emulsions. The color formers employed are of the type capable of forming azomethine, quinoneimine or azine dyes on color development, i.e., they contain a phenolic hydroxy or reactive methylene group, are oil soluble and preferably contain an aliphatic chain of at least 10 carbon atoms. Illustrative of color formers in this category are those described in Schneider et al., U.S.P. 2,186,849, without, however, a water solubilizing group being present in the color former molecule. The non-aqueous packets thus obtained are then dispersed in an aqueous solution of a water permeable colloid, such as gelatin, gum arabic, starch, polyvinyl alcohol, or carboxymethyl cellulose, with or without the aid of dispersing agents, as the occasion may demand and the operator may see fit to use. There are thus obtained stabilized, highly light sensitive dispersions, wherein the individual packets have no tendency to coalesce and function completely as individual entities. Preferably, the water soluble carrier should be capable of gelation so that once cast or gelled, a rigid matrix is obtained.

The applicability of this system to the formation of mixed grain photographic materials is self-evident. Thus,

this procedure would permit the separate sensitization of hydrophobic grains to the blue, green and red region of the spectrum along with color formers capable of giving a dye complementary in color to that of the spectral region to which the grains are sensitized.

The different packets may then be dispersed in one and the same water permeable colloid and the resulting emulsion coated and dried. Inasmuch as the various packets function as individual entities, a single exposure and color development with a primary aromatic amino developer such as the N-dialkyl-p-phenylenediamines, i.e., N-diethyl-p-phenylenediamine, 3-methyl-4-diethylaminoaniline, N- $\beta$ -hydroxyethyl-N-ethyl-p-phenylenediamine and the like would produce images in the various primary colors with adequate color separation being assured.

Our system lends itself readily to the formation of variable contrast emulsions. Here again, the immobility of the differently sensitized particles permits two different sets of silver halide grains in one and the same layer to function independently of each other.

Our emulsions, being non-aqueous, are less subject to degeneration on storage in areas of high humidity. This is an important aspect, particularly with regard to such high speed photographic film as X-ray and the like, and our system, therefore, recommends itself in the production of these materials.

Aside from its many different fields of application, our procedure has other important advantages. One of these is the ease with which dispersions of the non-aqueous emulsions can be made in aqueous media. Such dispersions are obtained by relatively mild stirring and energetic devices, such as colloid mills or other high energy mills, are unnecessary. Since only low energy dispersing machines are required, the dispersion can be accomplished without adversely affecting the photographic properties of the silver halides.

A further advantage resides in the fact that a drastic discontinuity between the packet and the matrix helps to isolate each individual packet and make it independent of chemical processes which may be taking place in an adjacent packet. Furthermore, it is possible to prepare packets of uniform size distribution and of almost any specified size.

The invention is further illustrated by the accompanying self-explanatory drawing, Figure I of which indicates the distribution of silver halides in an emulsion according to our invention, and Figure II of which discloses the distribution of silver halides in an emulsion, prepared in the same manner as that of Figure I, but in which the treatment to impart hydrophobic character to the silver halide grains is eliminated.

The following examples will serve to amplify the specific procedure contemplated, but it is to be understood that the invention is not restricted thereto.

#### DIGESTION PROCEDURE

##### Example I

500 grams of a silver chloride gelatin emulsion were melted at 40° C., after which 50 ml. of a 1% solution of polydase were added. Hydrolysis was complete in one hour at the above temperature. The reaction mixture was then allowed to stand a few hours at room temperature in order for the silver chloride to settle. The upper, clear digested gelatin was then decanted and the precipitate washed down twice with 200 ml. portions of 50% acetone (by volume) followed by two washings with 100% acetone, using 150 ml. of solvent each time. The washes were removed by decantation. The silver halide may then be made hydrophobic as subsequently described.

##### Example II

To 1000 grams of a melted gelatin silver halide were added 100 ml. of 1% trypsin as in Example I. After

removal of the digested gelatin, the precipitated silver halide was washed with two 200 ml. portions of 50% ethanol followed by two washings with 95% alcohol, using 150 ml. each time. The product was then made hydrophobic as subsequently described.

#### HYDROPHOBIZING STAGE

##### Example III

The silver halide isolated by enzymatic digestion as in Example I was suspended in a solution of 2.5 grams of myristic anhydride dissolved in 100 ml. of acetone. The mixture was tumbled in a small roller mill for several hours and then allowed to stand until the silver halide had settled. The acetone solution was decanted and the precipitate washed with two 150 ml. portions of fresh acetone. The damp cake was suspended in 30 ml. of phenyl ethyl alcohol and stirred vigorously for 3 minutes in a small Waring blender. The resulting milky oil containing the hydrophobic silver halide is ready to be incorporated in "packet" or "mixed grain" photographic emulsions.

##### Example IV

The silver halide obtained according to Example I was stirred up with a solution of 5.0 grams of myristic isocyanate in 100 ml. of acetone for 10 hours. The suspension was allowed to settle and the precipitate washed twice with 200 ml. portions of acetone. The damp cake of hydrophobic silver halide was then dispersed in tricresyl phosphate to be used in the preparation of mixed grain photographic emulsions.

##### Example V

The silver halide isolated by the procedure of Example II was suspended in a solution of 2.5 grams of myristoyl chloride in 100 ml. of acetone. After tumbling for 10 hours, the precipitate was allowed to settle and the acetone solution of acylating agent decanted. The product was then washed with two portions of acetone, using 200 ml. of solvent for each washing. The damp cake of hydrophobic silver halide was next thoroughly mixed with 25 ml. of benzyl alcohol and the resulting suspension employed in the preparation of mixed grain emulsion layers.

##### Example VI

The procedure was the same as in Example III, excepting that the hydrophobic character was imparted to the silver halide grains by treatment with octadecyl chlorocarbonate.

##### Example VII

The procedure was the same as in Example V, excepting that tetradecylsulfonyl chloride was employed to render the silver halide grains hydrophobic.

#### PREPARATION OF MIXED GRAIN DISPERSIONS

##### Example VIII

0.60 gram of 25% phenyl ethyl alcohol silver halide suspension prepared according to Example III was added to 30 ml. of 10% gelatin and the resulting mixture stirred vigorously for 5 minutes. A dispersion was obtained consisting of minute oily droplets, 2 to 4 microns in diameter containing embedded hydrophobic silver halide crystals.

##### Example IX

0.0683 gram of 1-phenyl-3-(10-undecenoylamino)-5-pyrazolone and .007 mg. of a green sensitizing dye were dissolved in a mixture of 2.0 grams of tricresyl phosphate plus 2.0 grams of phenyl ethyl alcohol by warming on the steam bath. Next was added 0.274 gram of a 24% hydrophobic silver chloride-benzyl alcohol suspension prepared according to Example V and the whole thoroughly mixed and stirred up in 30 ml. of 10% gelatin until particles ranging between 5 to 10 microns were obtained.

#### Example X

0.0902 gram of yellow coupler ( $N^4$ -acetyl-4'-benzoylacetamidosulfanilamide) was dissolved in a mixture of 2.0 grams of tricresyl phosphate plus 2.0 grams of benzyl alcohol to which was added 0.274 gram of 24% hydrophobic silver chloride suspended in phenyl ethyl alcohol and the whole mixed thoroughly. This mixture was then dispersed in 30 ml. of 10% gelatin until particles measuring 5 to 10 microns were obtained.

#### Example XI

To 0.0764 gram of 1-hydroxy-N-myristyl naphthamide and .007 mg. of a red sensitizing dye dissolved in a mixture of 1.0 gram of phenyl ethyl alcohol plus 1.0 gram of the product sold by Atlas Powder Company as "Span 80" was added with good stirring 0.274 gram of 24% hydrophobic silver chloride suspended in phenyl ethyl alcohol. This mixture was then dispersed in 30 ml. of 10% gelatin by stirring until the size of the droplets were 5 to 10 microns.

#### Example XII

To 0.0882 gram of 1-phenyl-3-stearoylamino-5-pyrazolone and .01 mg. of a green sensitizing dye dissolved in a mixture of 5.71 grams of phenyl ethyl alcohol, 0.67 gram of tricresyl phosphate and 0.08 gram of  $N$ -butyl phthalate was added 0.545 gram of 20.9% hydrophobic silver chloride suspended in phenyl ethyl alcohol. This mixture was thoroughly stirred and then dispersed in 30 ml. of 10% gelatin until particles measuring 5 to 10 microns in diameter had resulted.

#### Example XIII

To 0.152 gram of yellow coupler (4'-benzoylacetamido- $N^4$ -caproylsulfanilamide) dissolved in a mixture of 5.71 ml. of phenyl ethyl alcohol and 0.63 ml. of tricresyl phosphate was added 0.397 gram of 34.5% hydrophobic silver chloride phenyl ethyl alcohol suspension and the whole thoroughly stirred. This mixture was dispersed in 30 ml. of a 10% solution of gelatin in a small Waring blender. Agitation was continued until a particle size of 5 to 10 microns was achieved.

#### MIXED GRAIN DISPERSIONS

##### Example XIV

One part of the emulsion from Example IX was added to one part of the emulsion from Example XI, and the resulting mixture gently stirred for 5 minutes. This mixed emulsion was coated on suitable film base, dried and exposed through a step wedge and developed in a developing solution of the following composition to form a negative colored image:

|    |                                                            |       |       |
|----|------------------------------------------------------------|-------|-------|
| 55 | $N$ - $\beta$ -hydroxyethyl- $N$ -ethyl-p-phenylenediamine | grams | 5.0   |
|    | Sodium sulfite                                             | do    | 5.0   |
|    | Sodium carbonate .3H <sub>2</sub> O                        | do    | 120.0 |
| 60 | Potassium bromide                                          | do    | 1.0   |
|    | Ethylene diaminetetraacetic acid                           | do    | 0.8   |
|    | $\beta$ -Phenylethyl amine                                 | do    | 1.0   |
|    | Water to make 1000.0 cc.                                   |       |       |

Separate cyan and magenta images were obtained.

##### Example XV

One part of the green sensitive emulsion prepared in Example XII was added to one part of the blue sensitive emulsion from Example XIII. The mixture was gently agitated for 3 minutes and then coated on suitable film base and exposed through a blue and green filter. Development was carried out as described in Example XIV. Satisfactory color separation of magenta and yellow images was obtained in the portions of the coating exposed to green and blue light, respectively.

## Example XVI

To 0.152 gram of yellow coupler (4'-benzoylacetamido-N<sup>4</sup>-caproylsulfanilanilide) dissolved in a mixture of 5.71 ml. of phenyl ethyl alcohol and 0.63 ml. of tricesyl phosphate was added 0.397 gram of 34.5% hydrophobic silver chloride phenyl ethyl alcohol suspension and the whole thoroughly stirred. This mixture was dispersed in 30 ml. of a 7% solution of polyvinyl alcohol in a small Waring blender. Agitation was continued until a particle size of 5 to 10 microns was achieved.

## Example XVII

One part of the emulsion from Example IX, one part of the emulsion from Example X and one part of the emulsion from Example XI were added together and the resulting mixture gently stirred for a period of 5 minutes. The mixed emulsion was coated on a film base, dried, and exposed through a step wedge and developed in a solution of the following composition:

|                                    |       |       |
|------------------------------------|-------|-------|
| 3-methyl-4-diethylamino aniline    | grams | 5.0   |
| Sodium sulfite                     | do    | 5.0   |
| Sodium carbonate 3H <sub>2</sub> O | do    | 120.0 |
| Potassium bromide                  | do    | 1.0   |
| Ethylene diaminetetraacetic acid   | do    | 0.8   |
| β-Phenylethyl amine                | do    | 1.0   |
| Water to make 1000.0 cc.           |       |       |

Separate negatives of yellow, cyan and magenta images were thus obtained.

## Example XVIII

The procedure is the same as in Example XIV, excepting that the color developing agent is N-diethyl-p-phenylenediamine.

Our invention, while particularly adapted for mixed grain emulsion work, may also be used to produce multi-layer photographic color film of the conventional type. Thus, a base may be coated sequentially with a red sensitized emulsion (Example XI), a green sensitized emulsion (Example IX) and a blue sensitive emulsion (Example X). This monopack film layer may be exposed and processed with the usual primary aromatic amino color developers to the three complementary colored images.

We claim:

1. A light-sensitive photographic emulsion comprising a hydrophilic colloid carrier having dispersed therethrough immobile packets of an oily, non-water miscible solvent surrounding light-sensitive silver halide grains which have been rendered hydrophobic by treating a light-sensitive gelatin silver halide photographic emulsion with a proteolytic enzyme in order to digest the gelatin carrier and produce silver halide grains each surrounded by a hull of adsorbed gelatin, separating the light-sensitive grains and their adsorbed gelatin hulls from the digested gelatin and treating by intimately associating the gelatin hulls and said grains with an aliphatic compound

having a hydrocarbon chain of at least 10 carbon atoms and a substituent selected from the group consisting of acid anhydrides, acid chlorides, sulfonyl chlorides, isocyanates and chlorocarbonates.

5. The process of rendering silver halide grains hydrophobic which comprises treating a light-sensitive gelatin silver halide photographic emulsion with a proteolytic enzyme in order to digest the gelatin carrier and produce silver halide grains each surrounded by a hull of adsorbed gelatin, separating the light-sensitive grains and their adsorbed gelatin hulls from the digested gelatin and treating by intimately associating the gelatin hulls and said grains with an aliphatic compound having a hydrocarbon chain of at least 10 carbon atoms and a substituent selected from the group consisting of acid anhydrides, acid chlorides, sulfonyl chlorides, isocyanates and chlorocarbonates.

10. The emulsion as defined in claim 1, wherein certain of said silver halide grains are sensitized to one region of the spectrum and certain others are sensitized to a different region of the spectrum.

15. The emulsion as defined in claim 1, wherein certain of said silver halide grains are sensitized to the red region of the spectrum and have an oil soluble cyan color former associated therewith, others are sensitized for the green region of the spectrum and have an oil soluble magenta color former associated therewith, and others are sensitized to the blue region of the spectrum and have an oil soluble yellow color former associated there-  
20 with each of said color formers being capable of coupling with the oxidation product of an aromatic primary amino developing agent to form a dye.

25. The emulsion as defined in claim 1, wherein the colloidal carrier is water permeable.

30. The emulsion as defined in claim 4, wherein the color formers contain an aliphatic chain of at least 10 carbon atoms.

35. The process of producing subtractive multicolor dye images in a single layer of a photographic emulsion, which comprises exposing a single layer of the emulsion of claim 4 coated on a base and developing the same in an N-dialkyl-p-phenylenediamine developer.

## References Cited in the file of this patent

## UNITED STATES PATENTS

|              |                   |                |
|--------------|-------------------|----------------|
| 2,527,261    | Hart et al.       | Oct. 24, 1950  |
| 2,544,640    | Checkak           | Mar. 13, 1951  |
| 2,618,553    | Baines et al.     | Nov. 18, 1952  |
| 50 2,698,794 | Godowsky          | Jan. 4, 1955   |
| 2,728,662    | Yutzy et al.      | Dec. 27, 1955  |
| 2,763,552    | Van Campen et al. | Sept. 18, 1956 |
| 2,768,079    | Russell           | Oct. 23, 1956  |

## OTHER REFERENCES

Hamm: "Journal of Applied Physics," vol. 24, pp. 1495-1513, December 1953.